

Aug. 4, 1931.

S. G. MANDALIAN

1,817,519

MESH FABRIC

Filed Oct. 26, 1927



Fig. 1



Fig. 2



Fig. 3.

INVENTOR  
*Sahatiel G. Mandalian.*  
 BY  
*Koratoo E. Bellows*  
 ATTORNEY

## UNITED STATES PATENT OFFICE

SAMUEL G. MANDALIAN, OF NORTH ATTLEBORO, MASSACHUSETTS

## MESH FABRIC

Application filed October 26, 1927. Serial No. 228,885.

My invention relates to coated metallic mesh fabrics. These fabrics are of "link" mesh or "coat of mail" or "armor" mesh, and are initially cleaned and usually plated with precious metal.

Such plated mesh fabrics have heretofore been coated with a single layer of colored enamel having a base of oil and resin which required baking, and was not only frangible and subject to chipping by use, but tended to oxidize the material to which the coating was applied.

The objects of my invention are to avoid the above indicated defects, and to produce a mesh which is tough, strong, permanent, and infrangible throughout, and one in which the color is permanent or non fugitive and non fadable.

To the above ends essentially my invention consists in the means of securing the desired ends which fall within the scope of the appended claims.

In the drawings which form a part of this specification

25 Figure 1 is a plan view of an armor mesh fabric,

Figure 2, a section of a cruciform link taken on line 2—2 of Figure 1, and

30 Figure 3, a section of a ring link taken on line 3—3 of Figure 1.

Like characters of reference indicate like parts throughout the views.

The form of mesh herein illustrated comprises parallel rows of circular or ring links 35 4. Each four of which are engaged with a flat cruciform link or plate 5 by four corner prongs 6 converging in the rear of the plate. The links are of metal, and are initially cleaned and usually plated with a 40 metal by the electrolytic or other process.

The mesh has applied to its surface, preferably by an air or other brush, a coat of what may be characterized as a pyroxylin enamel or pyroxylin base lacquer enamel, in 45 distinction from an oil base enamel or a burnt on silicious vitreous type of enamel. In this the vehicle of the pigment is a pyroxylin base, namely nitro cellulose, and is quick drying by evaporation. A more 50 extended characterization of this pyroxylin

enamel or lacquer enamel is a pigment ground into a vehicle consisting primarily of nitrated cotton dissolved in suitable solvents, and may or may not include the incorporation of gums, resins or oils, and may or may not include plasticizers or softeners and sundry solvents or diluents.

Improved effects may be obtained by applying to the described pyroxylin enamel a top coating of a high grade clear lacquer (in distinction from a pigmented lacquer). A clear lacquer may be defined as substantially a solution of a nitrated cotton in a suitable solvent mixture, and may or may not include gums, resins or oils, or may or may not include plasticizers or softening agents, and sundry non solvents or diluents.

If desired the original coating of the plated mesh fabric may consist of a mixture created by the incorporation of varying proportions of clear lacquer in the pyroxylin enamel.

The above coat or coats are applied preferably by a brush, and quickly evaporates leaving a clear color, and when "clear" lacquer is used, a high gloss. The setting of the coat or coats by evaporation rather than by baking is an important time saver in my process, and the elimination of baking prevents the change of coloring occasioned by high temperatures. The avoidance of the necessity of baking results in an absence of any chemical reaction in the setting of the lacquer. As there is no chemical reaction in the setting of the pyroxylin enamel coating, the latter is more durable and the range of colors therein greater.

Over the described coating or coatings is applied by a brush or otherwise a finishing film or coating consisting of a mixture of pearl essence with a high grade clear cotton lacquer. Pearl essence is a suspension of the natural crystals of guanin in a liquid. In this instance the essence is of a pasty constituency and the clear lacquer is a thinner. This coating imparts a somewhat iridescent effect to the color and gloss of the earlier coat or coats.

In Figures 2 and 3, upon the bodies 7 and 8 of the links 5 and 4 respectively, are dis-

grammatically shown the layer or coating 10 of pyroxylin enamel or pyroxylin base lacquer enamel, superposed upon which is the coating or layer 11 of high grade clear lacquer, covered in turn with the layer 12 of pearl essence.

The resultant mesh is thus encased in a covering which is exceedingly tough, permanent and beautiful in color and finish, and non perishable in texture.

It will be understood that the use of the pearl essence lacquer coat should not be attempted upon a prior coat of "baked" or "oil base" enamel. This is because it is generally true that the mixture of the solvents and diluents used in the production of pyroxylin base products have a solvent or disintegrating action upon the films produced from oil base types of finishing materials.

The present application is a co-pending case with applicant's companion application Serial Number 228,864 which relates to the process for producing articles claimed in the present case.

I claim:—

1. As an improved article of manufacture, a metallic mesh fabric comprising links, a base layer of pyroxylin enamel thereon, and final layers of pearl essence supported by the base layer.

2. As an improved article of manufacture, a metallic mesh fabric comprising links, a base layer of pyroxylin base lacquer enamel, a secondary layer of high grade clear lacquer upon the first layer, and a layer of pearl essence upon the second layer.

3. As an improved article of manufacture, a metallic mesh fabric carrying a base layer of pyroxylin lacquer and a final layer of clear lacquer carrying pearl essence.

4. In a process for ornamenting metallic mesh fabric, the steps consisting in applying to the fabric a coat of a base lacquer containing pigmented pyroxylin and superposing thereon a clear pyroxylin lacquer.

In testimony whereof I have affixed my signature.

SAHATIEL G. MANDALIAN.